

## UNITED STATES PATENT OFFICE

2,448,479

URANIUM MONOCARBIDE AND METHOD OF  
PREPARATION

Harley A. Wilhelm and Adrian H. Daane, Ames,  
Iowa, assignors to the United States of America  
as represented by the United States Atomic  
Energy Commission

No Drawing. Application September 6, 1944,  
Serial No. 552,932

3 Claims. (Cl. 23—208)

1

This invention relates generally to uranium alloys and more particularly to uranium carbides. More specifically, our invention is concerned with the reduction of uranium oxides by carbon and the formation of uranium carbides of low carbon content, such as uranium monocarbide, UC, uranium dicarbide, UC<sub>2</sub>, and uranium sesquicarbide, U<sub>2</sub>C<sub>3</sub>, having less than about 10 per cent carbon. Uranium carbides of low carbon content have structural strength and resistance to wear superior to uranium metal or uranium oxide. In some applications of uranium forms these properties are desirable and the use of a uranium carbide is advantageous.

It is an object of our invention to provide a process for the preparation of uranium carbides of low carbon content and particularly the mono-, di-, and sesqui-carbides of uranium.

Another object is to provide a process for the production of these uranium carbides in massive form having a high density non-porous structure free of voids.

In the process of the present invention either uranium dioxide, (UO<sub>2</sub>) or uranium tritaoctaoxide (U<sub>3</sub>O<sub>8</sub>) may be used as a supply of uranium for the formation of uranium carbide. Uranium oxides are converted to uranium carbides by reaction with carbon at elevated temperatures, and we have found that a low concentration of carbon in a mixture with uranium oxide will reduce all of the oxide and form a carbide. The uranium carbides produced thereby may be the monocarbide, dicarbide, or sesquicarbide depending upon the proportions of constituents in the initial mixture.

Broadly, these uranium carbides of low carbon content may be prepared by first comminuting uranium oxide and carbon to a fine powder and mixing the two powdered substances, maintaining in the mixture a relatively low percentage of carbon. The powdered mixture may then be placed in a crucible and heated in a furnace to melting or nearly to melting causing a reaction of uranium oxide and carbon to take place whereby the desired carbide is produced accompanied by the evolution of carbon monoxide. The conversion of uranium oxide to low carbon uranium carbides may also be achieved by applying heat to a compressed mass. For example, the production of uranium carbides may be achieved by pressing the uranium oxide carbon mixture and then reacting the oxide and carbon in the compressed mass by heating it in the temperature range of from 1750° to 2375° C. and below the melting point of the uranium carbide formed.

2

The melting points of the uranium carbides are of the order of 2350° to 2400° C. for uranium dicarbide and uranium sesquicarbide, and 2250° to 2300° C. for uranium monocarbide. During this reaction the uranium oxide is reduced by the carbon and uranium carbide is formed. The heating of the pressed mass causes a sintering of the particles which causes the carbide produced to become more compact. The extent to which this sintering takes place depends upon the temperature and the period of heating, and the degree of sintering is increased by higher temperatures and longer heating periods. Therefore, the density of the uranium carbide produced is determined by the temperature at which the heating is carried on and the length of the period of heating. In general, it is preferable that the manufacture of uranium carbides be achieved from uranium dioxide, although uranium tritaoctaoxide may also be used to form carbides of low carbon content following the procedures outlined herein.

The carbon content of a uranium carbide formed by our process is directly related to the proportions of the components in the mixture of uranium oxide and carbon from which the carbide is produced. By ascertaining the relation between the quantitative ratio of the parts of uranium oxide and carbon in the initial mixture and the percentage composition of the uranium carbide produced, then it is possible to produce uranium carbide with a predetermined percentage of carbon by the selection of proper proportions of the components in the initial mixture.

We have discovered that in the formation of uranium carbides from uranium oxide by reduction with carbon, the quantities of oxide and carbon reacting with each other to form a particular carbide may be predetermined from the stoichiometric ratios of the chemical reaction involved, wherein all of the oxygen of the particular oxide used is converted into carbon monoxide. In forming a uranium carbide the reactants are mixed in about the stoichiometric ratio of the equation of the reaction for the particular carbide desired. As a result it is possible to predetermine the carbon percentage of the uranium carbide produced, by adjustment of the proportions of the oxide and carbon in the initial mixture.

As an example, uranium monocarbide may be formed by mixing uranium dioxide and carbon and heating this mixture. The production of the uranium monocarbide with its low carbon con-

tent is achieved by proportioning the parts of uranium dioxide and carbon in the reacting mixture, and by carrying on the reduction of the oxide by the carbon so as to reduce all the oxide with the formation of carbon monoxide and combine all the uranium and carbon, leaving no residual carbon or uranium dioxide. Uranium monocarbide is formed from uranium dioxide and carbon in conformance with the following equation:



In this reaction the reactants, uranium dioxide and carbon, have a stoichiometric ratio of 7.5 parts of uranium dioxide to one part of carbon by weight so that according to our invention, uranium dioxide and carbon when mixed in this proportion and heated to a temperature to cause reduction of the oxide will produce uranium monocarbide with the formula UC and with a carbon content of approximately 4.8 per cent.

In preparing uranium dicarbide from uranium dioxide and carbon according to the present invention, the reaction follows the equation:



In this equation the stoichiometric ratio of uranium dioxide to carbon in the initial mixture of the components is 5.626:1. The uranium dicarbide produced according to the above equation has a carbon content of about 9.16 per cent.

The preparation of uranium sesquicarbide from uranium dioxide and carbon by the process of the present invention follows the equation:



In this reaction the stoichiometric ratio of uranium dioxide to carbon is 6.43:1. When 6.4 parts of uranium dioxide are mixed with one part of carbon and heated according to this invention, the uranium sesquicarbide produced will have a carbon content of about 7.03 per cent.

The density and porosity of the mass of uranium carbide produced by melting or agglomerating can be varied and controlled by the particle size of the uranium oxide and carbon. The preparation of a uranium carbide from a mixture of uranium dioxide or uranium tritaoctaoxide is constituted by first grinding up and sieving the uranium oxide and the carbon and then mixing the powdered components. By grinding the uranium oxide and carbon to a powder that will pass fine mesh screens of the order of 100 mesh or finer, accurately shaped and less porous uranium carbide may be produced.

Where the conversion reaction is to take place in a carbon or graphite crucible, somewhat less than the stoichiometric percentage of carbon may be used in view of the fact that some of the crucible material may react with the uranium to form a carbide. It is also desirable in some cases to add extra uranium oxide to the crucible when the reaction between the carbon and uranium oxide of the original mixture is nearly complete.

The following examples illustrate specific embodiments of our invention as applied to the production of uranium carbides of low carbon content, but it is to be understood that similar results may be obtained by modified procedures without departing from the spirit of this invention.

*Example 1.*—7.5 parts by weight of uranium dioxide finely powdered to pass through a 100 mesh screen are mixed with one part of similarly fine graphite. The mixture is first pressed under about 26 tons per square inch to the form of a bar

1/2" x 1/2" x 2" having a density of 7 grams per cubic centimeter, and the bar is stood on end in a graphite crucible to prevent appreciable reaction of the mixture with the graphite of the crucible. The bar is then heated slowly to the range of 2275° C. to 2320° C., and the temperature maintained in this range for 20 minutes. An alloy with uranium and carbon in the ratio of  $\text{U}_1\text{C}_{1.27}$  is produced. This product is the compound UC containing some carbon dissolved or dispersed therein.

*Example 2.*—5.7 parts by weight of uranium dioxide powdered to pass a 100 mesh screen are mixed in an iron mortar with one part of graphite powdered to pass a 200 mesh screen. The mixture is inductively heated in a graphite crucible at about 9.5 kilowatts for 15 minutes and 12 kilowatts for 50 minutes. The product is a compact mass of uranium carbide having crystals radiating away from the center of the mass. Carbon analyses made on samples from this mass indicate an average of 9.15 per cent carbon which approximates the theoretical 9.16 per cent carbon in  $\text{UC}_2$ .

*Example 3.*—362.5 grams of graphite are mixed with 2037.5 grams of uranium dioxide and heated in a graphite crucible to a temperature between 2100° C. and 2300° C. while the conversion reaction takes place. After the reaction is completed, the temperature is raised to about 2500° C. The product is a mass of uranium dicarbide free of gas pockets and with a density measurement of 10.8 grams per cubic centimeter.

*Example 4.*—7.9 parts by weight of uranium dioxide powdered to pass a 100 mesh screen are mixed in an iron mortar with one part of graphite powdered to pass a 200 mesh screen. The mixture is heated in a pure graphite crucible, as much as possible being packed in at the beginning, and the remainder being added after the reaction begins. The heating is carried on at about 9.5 kilowatts for 15 minutes, and at about 12 kilowatts for 50 minutes. The product is a well formed mass which analyzes to give 7.21 per cent carbon indicating the formation of the dicarbide and the sesquicarbide.

*Example 5.*—8 parts by weight of uranium dioxide are mixed with one part of carbon. The mixture is heated in a crucible in an induction furnace to give a compact mass containing uranium sesquicarbide with an overall density of 11.5 grams per cubic centimeter.

*Example 6.*—7.5 parts by weight of uranium dioxide are mixed with one part of graphite. The mixture is heated in a crucible in an induction furnace. A mass including uranium sesquicarbide crystals is produced in a well-shaped form.

Although the reactions of uranium dioxide have been used to illustrate the application of the process of the present invention, other methods within the spirit of this invention may be used to obtain uranium carbides. Uranium dioxide may be melted in a graphite crucible, when heated quickly to avoid reaction with the crucible, and uranium dicarbide chunks added to the melt. The product is uranium dicarbide, due to the reaction of the uranium dioxide with the graphite of the crucible walls.

Thus we have been able, by following the process described and claimed herein, to consistently produce uranium-carbon alloys having a predetermined carbon content of less than about 10 per cent.

While the foregoing embodiments of our invention have been discussed as performed in an

air atmosphere, a hydrogen atmosphere has also been found suitable.

Numerous variations and modifications in the preferred methods and examples described will be readily apparent and may be made without departing from the spirit and scope of our invention as defined in the following claims.

We claim:

1. A method of forming uranium monocarbide which comprises heating to reaction temperature 10 a mixture comprising an oxide of uranium and carbon in substantially stoichiometric proportions required for monocarbide.

2. A method of forming uranium monocarbide which comprises heating to reaction temperatures a mixture comprising  $UO_2$  and carbon in substantially stoichiometric proportions required 15 for monocarbide.

3. Uranium monocarbide having the composition UC.

HARLEY A. WILHELM.  
ADRIAN H. DAANE.

#### REFERENCES CITED

The following references are of record in the file of this patent:

#### UNITED STATES PATENTS

| Number    | Name                | Date          |
|-----------|---------------------|---------------|
| 2,017,558 | Winter et al. ----- | Oct. 15, 1935 |
| 2,364,123 | Benner et al. ----- | Dec. 5, 1944  |

#### OTHER REFERENCES

15 Chemical Abstracts, vol. 8 (1914), article by Tiede et al., page 2855, line 11.